

## UNITED STATES PATENT OFFICE.

CHARLES F. BOOTH AND ARTHUR B. GERBER, OF ANNISTON, ALABAMA, AND PAUL LOGUE, OF LOGUE, MISSOURI.

## SALINE TRI-SODIUM PHOSPHATE AND PROCESS FOR ITS MANUFACTURE.

No Drawing. Refiling of application Serial No. 726,919, filed July 19, 1924. This application filed June 25, 1928. Serial No. 288,287.

This invention relates to a process for the manufacture of compounds of alkali-metal phosphate and particularly to the manufacture of a sodium chloride tri-sodium phosphate compound such as referred to in our co-pending application, Serial No. 726,920.

The object of this invention is to produce a compound requiring in its manufacture less caustic than is now used in the manufacture of commercial tri-sodium phosphate. It follows that the material provided by our present process will contain less free caustic and be less injurious to fabrics and to individuals handling it.

According to the present practice, tri-sodium phosphate is generally manufactured by the neutralization of sodium carbonate, which is commercially called soda ash, with phosphoric acid, whereby di-sodium phosphate is produced. After the production of di-sodium phosphate, it is causticized by the addition of caustic soda, thus converting the di-sodium phosphate into tri-sodium phosphate. The resultant tri-sodium phosphate solution is then cooled in a suitable manner and solid tri-sodium phosphate separated out as a crystalline material. Based on the following chemical equations:



the theoretical quantities of materials necessary for the production of tri-sodium phosphate are as follows:

25.7#  $\text{H}_3\text{PO}_4$  per 100# tri-sodium phosphate.

27.8#  $\text{Na}_2\text{CO}_3$  per 100# tri-sodium phosphate.

10.5# NaOH per 100# tri-sodium phosphate.

Actual practice from several years' operation shows that in so far as the caustic is concerned this quantity is insufficient, and as a result of this increased caustic consumption it appears that the material which is commercially called tri-sodium phosphate does not conform to the formula  $\text{Na}_3\text{PO}_4 \cdot 12\text{H}_2\text{O}$  but contains in addition NaOH, and the caustic soda necessary for crystallization of

tri-sodium phosphate approaches nearer 15# than the theoretical 10.5# NaOH as given above. Extensive experiments were conducted to determine if it were possible to reduce the quantity of caustic necessary in tri-sodium phosphate manufacture as that element is both expensive and objectionable. During this investigation it was discovered that it was possible to produce tri-sodium phosphate by the use of less caustic soda, and the resulting compound having a "ratio" of 0.50 when titrated with a standard acid, using phenolphthalein and methyl orange as indicators. We have found that a different compound can be produced from this neutral tri-sodium or di-sodium phosphate solution by the addition of sodium chloride, the addition of which to the tri-sodium or di-sodium phosphate solution improved the crystallization of the tri-sodium phosphate compound. This invention relates to the process by which a sodium chloride tri-sodium phosphate compound is produced in connection with the above mentioned sodium salt.

After considerable experimental work in the effort to increase the size of crystals of the tri-sodium phosphate produced as described, in applications, Serial Nos. 726,917 and 726,918, filed July 19, 1924, by A. B. Gerber and C. F. Booth, it was found that by the addition of common salt (NaCl), it was possible to produce materials having all the desirable characteristics of the alkaline or commercial tri-sodium phosphate as found on the market at present; also, the large quantity of caustic required for the production of the latter was unnecessary. It was also found that the new material thus produced did not have the same harsh caustic drying action on the skin as the alkaline or commercial tri-sodium phosphate as found on the market at present. In addition to these features the reduced caustic requirement was of considerable advantage so far as the cost of production was concerned, because it is possible to make this new compound with approximately the theoretical requirement of caustic soda. While the exact composition of this compound is not fully understood, it is believed a molecular compound in which the NaOH of alkaline or commercial tri-sodium phosphate is replaced by the sodium

chloride. For instance, the compound is believed to have a formula



- 5 This opinion is based on the fact that the crystals have a "ratio" about 0.50 and contain about 3% NaCl. This caustic soda requirement or "ratio" in producing solutions for crystallization may be judged by a method of control in which the sodium chloride tri-sodium phosphate solution is titrated with a half normal hydrochloric acid solution using phenolphthalein and methyl orange as indicators.
- 15 When the end point for the phenolphthalein is reached, a reading is made of the acid used, and the titration is continued to a slight acid end point with the methyl orange. The reading of the titration of the phenolphthalein is then divided by the sum of the readings, and a "ratio" of 0.46 to 0.50 is the desired resultant for the optimum conditions to produce the best yield of sodium chloride tri-sodium phosphate crystals when 25 the solution is cooled. The "ratio" so determined is one means of deriving a constant as a measure of the caustic present in the solution or crystals. Where the term "ratio" is used herein it refers to such method of 30 determination of the relation of phenolphthalein end point to methyl orange indicator end point in the solution of sodium chloride tri-sodium phosphate or crystals thereof. It will therefore be seen that the production 35 of this new compound by our process, offers distinct economic advantages over the manufacture of alkaline or commercial tri-sodium phosphate as produced at the present time, and in addition to this economic feature, a 40 sodium chloride tri-sodium phosphate compound is produced which has distinct advantages for the consumer.

The process and equipment of manufacture is similar to that carried on and used 45 in the manufacture of alkaline or commercial tri-sodium phosphate as found on the market at present. According to our process, phosphoric acid is neutralized by adding sodium carbonate ( $\text{Na}_2\text{CO}_3$ ) to di-sodium 50 phosphate and 4% sodium chloride (NaCl) is added to the di-sodium phosphate solution. After the sodium chloride addition, the necessary caustic is added to conform 55 approximately to the requirement as given in the chemical equation as follows:



The amount of sodium chloride varies according to the titration "ratio", more sodium chloride being required with a high "ratio". The titration "ratio" varies from approximately 0.46 to 0.50, depending upon the concentration of the solution, a high "ratio" being used for higher concentrations.

After the sodium chloride tri-sodium phosphate solution is tested as described above, it is cooled in any suitable manner and the sodium chloride tri-sodium phosphate crystals separate out. They may be dried in a 70 centrifuge or any other suitable means of dewatering, and then steam or air dried to remove the surface moisture. After drying, the crystals are ready for shipment.

The following proportions are given as 75 illustrative of the mixture required in making the above described sodium chloride tri-sodium phosphate compound by our process:—

43# 60%  $\text{H}_3\text{PO}_4$  (25.8#  $\text{H}_3\text{PO}_4$ )  
28# commercial soda ash (58%  $\text{Na}_2\text{O}$ )  
11# caustic soda (76%  $\text{Na}_2\text{O}$ )  
8# sodium chloride.

The acid is neutralized by the soda ash and any impurities such as iron, alumina, 85 and calcium phosphates which are precipitated, are removed from the solution, preferably by filtration. The di-sodium phosphate solution is boiled prior to filtration in order that the carbon dioxide ( $\text{CO}_2$ ) may be 90 eliminated. After filtration salt and caustic soda are added and the solution thoroughly mixed. The mixture is then tested according to the previously outlined method and if sufficient caustic has not been added, an addition is made until the titration gives the desired figure; while if an excess of caustic has been added, di-sodium phosphate solution is added to reduce the figure to the desired point. The same requirement can be 100 used for the subsequent cooling, crystallization, dewatering and drying of this product as for the alkaline or commercial tri-sodium phosphate as found on the market at present. When we refer to alkaline or commercial tri-sodium phosphate, as found on the market at present, we mean to include its compounds, whatever the composition may be.

Having thus described our invention, what we claim as new and desire to secure by Letters Patent, is:—

1. The herein described process for the manufacture of a sodium chloride tri-sodium phosphate composition, which consists in combining phosphoric acid, sodium carbonate, and caustic soda with sodium chloride and water.

2. The herein described process for the manufacture of a sodium chloride tri-sodium phosphate composition, which consists in combining concentrated phosphoric acid, sodium carbonate, and caustic soda with sodium chloride and water and cooling the solution and separating out the sodium chloride tri-sodium phosphate composition in crystalline form.

3. The herein described process for the manufacture of a sodium chloride tri-sodium phosphate composition, which consists in combining phosphoric acid, sodium carbon-

- ate, and caustic soda solution with sodium chloride and water, and separating out the crystalline product.
4. The herein described process for the manufacture of a sodium chloride tri-sodium phosphate composition, which consists in the addition of sodium chloride and caustic soda to di-sodium phosphate, substantially as described.
5. The herein described process for the manufacture of a sodium chloride tri-sodium phosphate composition, which consists in the addition of sodium chloride and caustic soda solutions to di-sodium phosphate solution, substantially as described.
10. The herein described steps in the process for the manufacture of a sodium chloride tri-sodium phosphate composition, which consists in the neutralization of phosphoric acid with sodium carbonate, removing all solids thus formed, and adding sodium chloride and caustic soda, substantially as described.
15. The herein described steps in the process for the manufacture of a sodium chloride tri-sodium phosphate composition, which consists in neutralizing dilute phosphoric acid with sodium carbonate, removing all solids thus formed, concentrating the di-sodium phosphate solution, and adding sodium chloride and caustic soda, substantially as described.
20. The herein described steps in the process for the manufacture of a sodium chloride tri-sodium phosphate composition, which consists in neutralizing concentrated phosphoric acid with sodium carbonate, removing all solids thus formed, concentrating the solution, adding sodium chloride and caustic soda, and cooling and crystallizing the so-
- dium chloride tri-sodium phosphate composition, substantially as described.
25. The herein described process for the manufacture of a sodium chloride tri-sodium phosphate composition, which consists in adding sodium chloride and caustic soda to di-sodium phosphate solution, concentrating the solution, and cooling and crystallizing a sodium chloride tri-sodium phosphate composition therefrom, substantially as described.
30. The herein described composition of matter consisting of a compound of sodium phosphate and sodium chloride.
35. Therein described composition of matter consisting of a compound of tri-sodium phosphate and sodium chloride.
40. The herein described composition of matter consisting of sodium phosphate and sodium chloride in a crystalline form.
45. The herein described composition of matter consisting of tri-sodium phosphate and sodium chloride in a crystalline form.
50. The herein described composition of matter consisting of a compound of sodium phosphate and sodium chloride.
55. The herein described composition of matter consisting of sodium phosphate and sodium chloride in a crystalline form.
60. The herein described composition of matter consisting of tri-sodium phosphate and sodium chloride in a crystalline form.
65. The herein described composition of matter consisting of tri-sodium phosphate and sodium chloride containing approximately 18.8%  $P_2O_5$ .
70. The herein described crystalline sodium phosphate composition crystallized from a sodium phosphate solution containing approximately 4% sodium chloride.

In testimony whereof we affix our signatures.

CHARLES F. BOOTH.  
ARTHUR B. GERBER.  
PAUL LOGUE.